

## UNITED STATES PATENT OFFICE

2,196,754

## TREATING CELLULOSE DERIVATIVE MATERIALS

Joseph B. Dickey and James G. McNally, Rochester, N. Y., assignors to Eastman Kodak Company, Rochester, N. Y., a corporation of New Jersey

No Drawing. Application December 17, 1938,  
Serial No. 246,517

7 Claims. (Cl. 28—1)

This invention relates to the conditioning of textile yarns and more particularly to the conditioning of filaments and yarns composed of organic derivatives of cellulose such as cellulose acetate, cellulose propionate, cellulose acetate propionate, and cellulose acetate butyrate, to render them more amenable to textile operations such as knitting and the like. This invention also relates to compositions of matter in which cellulose derivatives, such as cellulose acetate, cellulose nitrate or cellulose ethers, are combined or mixed with other substances, such as a compatible plasticizer, and a common solvent for both, with or without other useful addition agents, so that the resulting product will have properties such as will make the composition highly advantageous for use in the plastic and analogous arts, such for instance, as the manufacture of wrapping sheets, photographic film, artificial silk, varnishes or lacquers, and the like.

As is well known in the manufacture of yarns, particularly those composed of or containing cellulose organic derivatives, it is necessary to treat the yarn in order to reduce the tendency toward breakage of the individual filaments or fibers when they are subjected to various mechanical strains and to lubricate the yarn in order to facilitate handling in such operations as spinning, twisting, winding and reeling. It is also necessary to treat yarn to adapt it for use as warp or filling or for the manufacture of various types of knitted fabrics. In knitting, it is particularly important that the yarn be soft and pliable in order that it may conform readily to the contour of the needles and thus produce a closely knit fabric free from such defects as "stitch distortion", "pin holes", "laddering", and the like.

Heretofore it has been proposed to employ softening agents such as polyhydric alcohols and similar agents as ingredients of yarn conditioning or lubricating formulas, generally in connection with mineral, animal or vegetable oils. It has been found, however, that most of the known softening agents and the various formulas containing them have certain drawbacks, one of the most serious of which is high vapor pressure, and in some cases too drastic a solvent action on the yarn. Many of such agents possess slight or insufficient solvent power for the lubricants with which they are used, and it is accordingly necessary to employ blending agents or emulsifying agents in order to obtain operable yarn treating formulas. In addition, many of the known softening and lubricating agents are insufficiently

soluble in water to permit satisfactory removal by aqueous scour baths.

While in the plastic and related arts cellulose acetates, nitrates and ethers have been known for decades, it has also been known that to utilize them it is necessary to mix therewith such plasticizing or conditioning agents as camphor, castor oil, triphenyl phosphate, monochloronaphthalene or the like. Certain of these and other addition agents are also added for the purpose of reducing the inflammability of the product. Plastic inducing agents, such as the higher alcohols and their esters, are sometimes also added. Similarly, addition compounds of various kinds have been employed to increase flexibility, transparency, toughness, and other properties which will enhance the value of the resulting product. Addition products for the same or similar purposes are also added to cellulose acetates, nitrates and ethers to prepare them for use in the other plastic arts, such as in the manufacture of lacquers, varnishes, artificial silk filaments, moulded compounds and the like. While the plasticizers or other addition agents heretofore discovered have had their utility in the art, the increasing use to which cellulose derivatives have been put and the increasing number of desirable properties required of the cellulose derivative for most purposes has made the discovery of new and economical plasticizers or other addition agents a matter of considerable importance to the art.

This invention has as its principal object to provide an entirely new class of yarn conditioning agents which are particularly adapted for the treatment of yarns composed of or containing organic derivatives of cellulose and capable of lubricating, softening and rendering such yarns more amenable to knitting and other textile operations. A further and specific object is to provide a class of conditioning agents which augment or assist the lubricating action of various lubricants when applied to such yarns. A still further object is to provide yarn softening and lubricating formulas which can be readily removed from the yarns by the usual scour baths. A still further object is to provide an improved method for the conditioning of yarns, particularly those composed of or containing organic derivatives of cellulose such as cellulose acetate, whereby the yarn is rendered soft and pliable and capable of employment in a variety of textile operations where complicated designs or stitches are employed. Another object is to provide an improved type of yarn which is especially amenable to textile operations including circular knit-

20

25

30

35

40

45

50

55

ting, weaving, spinning and the like. Still another object of this invention is to produce a composition of matter which may be made into permanently transparent, strong and flexible sheets or films of desired thinness which are substantially waterproof, are unaffected by ordinary photographic fluids and possess the desired properties of a support for sensitive photographic coatings. Yet another object of our invention is to produce a composition which is capable of easy and convenient manipulation in the plastic and analogous arts, such as in the manufacture of sheets, films, artificial silk filaments, varnishes, lacquers and the like, and to produce a composition which will not injure, or be injured by, the substances or surfaces with which it is associated during manufacture. Other objects will appear hereinafter.

These objects are accomplished by the following invention which, in its broader aspects, comprises the discovery that esters of hydroxyalkoxy tetrahydrofurfuryl ethers having the general formula:



where  $n$  is a small whole number at least one;  $x$  is a small whole number at least one;  $B$  is a substituent selected from the group consisting of hydrogen, alkyl and hydroxy alkyl groups, and  $R$  is a substituent selected from the group consisting of the alkyl, cycloalkyl, aryl and heterocyclic groups, may be used as yarn conditioning agents and particularly as softening agents, with or without the addition of animal, mineral, or vegetable oils, in the treatment of yarns composed of or containing organic derivatives of cellulose. We have found that these compounds when employed as described in the detailed examples set forth below have a slight solvent and/or softening action on cellulose organic derivative yarns which renders such yarns soft and pliable without at the same time having too drastic an action thereon.

These compounds are prepared by treating hydroxyalkoxy tetrahydrofurfuryl ethers, which have the general formula



with acids, acid anhydrides and acid chlorides with or without the presence of a catalyst. These ethers may be prepared in accordance with the process set forth in my copending application Serial No. 246,205, filed December 16, 1938. When acids are used we may carry out the esterification in the presence of a catalyst such as sulfuric, phosphoric, p-toluene-sulfonic acid and remove the water formed by means of an azotropic mixture. We may use any type of organic acid such as butyric, methoxy acetic, oleic, malonic, adipic, citric, furoic, phthalic, tetrachlorophthalic, benzoic, benzene tricarboxylic, naphthenic, etc.

Our invention also comprises the discovery that valuable properties may be induced in and/or contributed to compositions containing cellulose derivatives such as cellulose acetate, by adding thereto as plasticizing compounds the above mentioned compounds. This class of compounds is compatible with cellulose derivatives

and particularly compatible with cellulose acetate in the percentages hereinafter given.

#### PREPARATION OF COMPOUNDS

##### Tetrahydrofurfuroxyethoxyethyl acetate 5

46 gm. of triethylene glycol tetrahydrofurfuryl ether and 30 gm. of acetic anhydride are refluxed for 1 hr. The product is then worked up to give the ester boiling 180-5°/0.1 mm.

##### Tetrahydrofurfuroxy ethyl butyrate 10

95 gm. of diethylene glycol tetrahydrofurfuryl ether and 90 gm. of butyric anhydride are heated on the steam bath for 1 hr. and then refluxed 5 minutes. The yellow product is then fractionated. The desired ether ester boils at 180-5°/15 mm.

##### Tetrahydrofurfuroxy ethyl tetrahydrofuroxy acetate 20

96 gm. of tetrahydrofuroxy acetic acid, 100 gm. of tetrahydrofuroxy ethanol, 0.3 gm. p-toluene sulfonic acid, and 150 cc. toluene are distilled so that the toluene returns to the reaction vessel. The theoretical quantity of water is collected during 6 hrs. The product is then washed with 10% sodium carbonate and distilled under vacuum. Toluene and the excess alcohol come off and then the ester, boiling 183-90°/3 mm.

##### Tetrahydrofurfuroxy ethyl succinate 30

35 gm. of succinic acid, 100 gm.  $\beta$  tetrahydrofurfuroxy ethanol, 0.2 g. p-toluene sulfonic acid, and 100 cc. benzene are refluxed in such a manner that the benzene separates from the water formed and returns to the reaction. After the necessary quantity of water has been collected, the product is washed with sodium carbonate solution (10%). The benzene and excess alcohol are removed and the ester distilled under vacuum. 47 gm. (70%) are obtained, boiling at 225-30°/3 mm.

The following table gives the constants of some of the compounds claimed in this sketch sheet.

|                                               | B. p.   | Pres-<br>sure |
|-----------------------------------------------|---------|---------------|
| Tetrahydrofuroxy ethyl acetate.....           | 152-6   | 50            |
| propionate.....                               | 138-43  | Mm.           |
| succinate.....                                | 225-30  | 18            |
| laurate.....                                  | 160-75  | 3             |
| oleate.....                                   | 210-50  | 0.1           |
| Tetrahydrofuroxy acetate.....                 | 183-90  | 3             |
| Tetrahydrofuroxy ethoxy ethyl butyrate.....   | 180-5   | 40            |
| acetate.....                                  | 195-200 | 15            |
| Tetrahydrofuroxy ethoxy ethyl butyrate.....   | 180-5   | 55            |
| acetate.....                                  | 170-5   | 0.1           |
| Tetrahydrofuroxy ethyl tetrahydrofuroate..... | 150-160 | 0.1           |

#### TREATMENT OF TEXTILE YARNS

In accordance with the invention these compounds may be applied directly to the yarn during or after spinning, or may be added to the spinning solution itself. We have found that these compounds have exceptional solvent powers which enable them to dissolve mineral oils and blown and unblown, drying and semi-drying, vegetable and animal oils and accordingly they may be, and preferably are, employed as ingredients of yarn conditioning or lubricating formulas in conjunction with agents which function wholly or partially as lubricants.

In the following examples and description we have set forth several of the preferred embodi-

ments of our invention, but they are included merely for purposes of illustration and not as a limitation thereof.

Our invention will be more readily understood by reference to the following examples in which typical applications of the invention are set forth.

*Example 1*

$\beta$ -hydroxy ethyl tetrahydrofurfuryl ether 10 oleate is applied to textile materials (silk, wool, cellulose acetate, cotton, viscose, etc.) by means of a wick, roller, spray, bath, pad, etc., to facilitate their knitting, weaving, spinning and the like. If the yarn is intended primarily for knitting the amount of conditioning liquid applied 15 may vary from 4-25% by weight of the yarn, and if the yarn is intended for weaving, the amount of liquid applied may vary between 1-5% by weight of the yarn.

*Example 2*

|                                                                                                                                                                                                                                                                          | Parts |
|--------------------------------------------------------------------------------------------------------------------------------------------------------------------------------------------------------------------------------------------------------------------------|-------|
| $\begin{array}{c} \text{H}_2\text{C} \text{---} \text{CH}_2 \\   \\ \text{CH}_2\text{---} \text{C} \text{---} \text{CH}_2 \text{---} \text{O} \text{---} \text{C}_2\text{H}_4 \text{---} \text{O} \text{---} \text{C} \text{---} \text{C}_{11}\text{H}_{23} \end{array}$ | 70    |
| ( $\beta$ -hydroxy- $\beta$ -ethoxy ethyl (6-methyl) tetrahydrofuran ether laurate)                                                                                                                                                                                      |       |
| Olive oil                                                                                                                                                                                                                                                                | 30    |

and applied to textile materials such as silk, wool, cotton, viscose, cellulose acetate, etc., as described in Example 1. If the yarn is intended primarily for knitting, the amount of conditioning liquid applied may vary from 4-25% by weight of the yarn, and if the yarn is intended for weaving, the amount of liquid applied may vary between 1-5% by weight of the yarn. Cellulose acetate filaments or fibers treated as described are quite soft and pliable and give improved results in various textile operations, such as weaving, knitting, etc.

Other examples of yarn conditioning compositions which may be applied to various types of yarns, particularly those composed of or containing cellulose acetate, cellulose acetate propionate, cellulose acetate butyrate, and similar cellulose organic acid esters in accordance with our invention and which render such yarns soft and pliable and especially well adapted for various textile operations, particularly knitting, are as follows:

*Example 3*

|                                                                                                                                                                                                                                                                                                                                                                                                             | Parts |
|-------------------------------------------------------------------------------------------------------------------------------------------------------------------------------------------------------------------------------------------------------------------------------------------------------------------------------------------------------------------------------------------------------------|-------|
| $\begin{array}{c} \text{H}_2\text{C} \text{---} \text{C} \text{---} \text{H}_2 \\   \\ \text{CH}_3\text{---} \text{CH}_2 \text{---} \text{C} \text{---} \text{O} \text{---} \text{CH}_2 \text{---} \text{C} \text{---} \text{CH}_2 \text{---} (\text{OCH}_2\text{---} \text{CH}_2)_2 \text{---} \text{O} \text{---} \text{C} \text{---} \text{CH}_2 \text{---} \text{O} \text{---} \text{CH}_2 \end{array}$ | 50    |
| ( $\beta$ -hydroxy- $\beta$ -ethoxy- $\beta$ -ethoxy-(5-omega-hydroxy methyl) tetrahydrofurfuryl ethyl ether bis methoxy acetate)                                                                                                                                                                                                                                                                           |       |
| Blown olive oil                                                                                                                                                                                                                                                                                                                                                                                             | 60    |

*Example 4*

|                                                                                                                                                                                                                                                                                                                                                                                                                                                                        | Parts |
|------------------------------------------------------------------------------------------------------------------------------------------------------------------------------------------------------------------------------------------------------------------------------------------------------------------------------------------------------------------------------------------------------------------------------------------------------------------------|-------|
| $\begin{array}{c} \text{H}_2\text{C} \text{---} \text{C} \text{---} \text{H}_2 \\   \\ \text{H}_2\text{C} \text{---} \text{CH}_2 \text{---} \text{O} \text{---} (\text{C}_2\text{H}_4)_2 \text{---} \text{O} \text{---} \text{C} \text{---} \text{C}_8\text{H}_{15} \text{---} \text{C} \text{---} \text{O} \text{---} (\text{C}_2\text{H}_4\text{---} \text{O})_2 \text{---} \text{O} \text{---} \text{CH}_2 \text{---} \text{CH} \text{---} \text{CH}_2 \end{array}$ | 55    |
| (bis( $\beta$ -hydroxy- $\beta$ -ethoxy- $\beta$ -ethoxy- $\beta$ -ethoxy tetrahydrofurfuryl ethyl ether) sebacate)                                                                                                                                                                                                                                                                                                                                                    |       |
| Light mineral oil                                                                                                                                                                                                                                                                                                                                                                                                                                                      | 60    |

*Example 5*

|                                                                                                                                                                                                                                                                                 | Parts |
|---------------------------------------------------------------------------------------------------------------------------------------------------------------------------------------------------------------------------------------------------------------------------------|-------|
| $\begin{array}{c} \text{H}_2\text{C} \text{---} \text{CH}_2 \\   \\ \text{H}_2\text{C} \text{---} \text{CH} \text{---} \text{CH}_2 \text{---} (\text{O} \text{---} \text{C}_2\text{H}_4)_5 \text{---} \text{O} \text{---} \text{C} \text{---} \text{C}_4\text{H}_9 \end{array}$ | 65    |
| ( $\beta$ -hydroxy- $\beta$ -ethoxy- $\beta$ -ethoxy- $\beta$ -ethoxy- $\beta$ -ethoxy tetrahydrofurfuryl ethyl ether valerate)                                                                                                                                                 |       |
| Blown sperm oil                                                                                                                                                                                                                                                                 | 30    |

*Example 6*

|                                                                                                                                                                                                                                                                                                                                   | Parts |
|-----------------------------------------------------------------------------------------------------------------------------------------------------------------------------------------------------------------------------------------------------------------------------------------------------------------------------------|-------|
| $\begin{array}{c} \text{H}_2\text{C} \text{---} \text{CH}_2 \\   \\ \text{H}_2\text{C} \text{---} \text{CH} \text{---} \text{CH}_2 \text{---} \text{O} \text{---} \text{C}_2\text{H}_4 \text{---} \text{O} \text{---} \text{C} \text{---} \text{C} \text{---} \text{O} \text{---} \text{CH}_2 \text{---} \text{CH}_2 \end{array}$ | 70    |
| ( $\beta$ -hydroxy ethyl tetrahydrofurfuryl ether furoate)                                                                                                                                                                                                                                                                        |       |
| Neat's-foot oil                                                                                                                                                                                                                                                                                                                   | 75    |

*Example 7*

|                                                                                                                                                                                                                                                                                | Parts |
|--------------------------------------------------------------------------------------------------------------------------------------------------------------------------------------------------------------------------------------------------------------------------------|-------|
| $\begin{array}{c} \text{H}_2\text{C} \text{---} \text{CH}_2 \\   \\ \text{H}_2\text{C} \text{---} \text{C} \text{---} \text{CH}_2 \text{---} (\text{O} \text{---} \text{C}_2\text{H}_4)_5 \text{---} \text{O} \text{---} \text{C} \text{---} \text{C}_6\text{H}_5 \end{array}$ | 20    |
| ( $\beta$ -hydroxy- $\beta$ -ethoxy ethyl tetrahydrofurfuryl ether benzoate)                                                                                                                                                                                                   |       |
| Blown teased                                                                                                                                                                                                                                                                   | 5     |
| Sulfonated soyabean oil                                                                                                                                                                                                                                                        | 30    |
| White mineral oil                                                                                                                                                                                                                                                              | 20    |
| Oleic acid                                                                                                                                                                                                                                                                     | 10    |
| Ethanolamine                                                                                                                                                                                                                                                                   | 10    |
| Water                                                                                                                                                                                                                                                                          | 7     |

*Example 8*

|                                                                                                                                                                                                                       | Parts |
|-----------------------------------------------------------------------------------------------------------------------------------------------------------------------------------------------------------------------|-------|
| $\begin{array}{c} \text{H}_2\text{C} \text{---} \text{CH}_2 \\   \\ \text{H}_2\text{C} \text{---} \text{C} \text{---} \text{CH}_2 \text{---} \text{O} \text{---} \text{C}_2\text{H}_4\text{---} \text{O} \end{array}$ | 20    |
| ( $\beta$ -Hydroxy- $\beta$ -ethoxy ethyl tetrahydrofurfuryl ether phthalate)                                                                                                                                         |       |
| Sperm oil                                                                                                                                                                                                             | 15    |
| Lauro                                                                                                                                                                                                                 | 20    |

*Example 9*

|                                                                                                                                                                                                                                                                             | Parts |
|-----------------------------------------------------------------------------------------------------------------------------------------------------------------------------------------------------------------------------------------------------------------------------|-------|
| $\begin{array}{c} \text{H}_2\text{C} \text{---} \text{CH}_2 \\   \\ \text{H}_2\text{C} \text{---} \text{CH} \text{---} \text{CH}_2 \text{---} \text{O} \text{---} \text{C}_2\text{H}_4 \text{---} \text{O} \text{---} \text{C} \text{---} \text{C}_6\text{H}_5 \end{array}$ | 20    |
| ( $\beta$ -Hydroxy ethoxy tetrahydrofurfuryl ether phenoxy acetate)                                                                                                                                                                                                         |       |
| Oleyl alcohol                                                                                                                                                                                                                                                               | 25    |
| Blown soyabean oil                                                                                                                                                                                                                                                          | 60    |

*Example 10*

|                                                                                                                                                                                                                                 | Parts |
|---------------------------------------------------------------------------------------------------------------------------------------------------------------------------------------------------------------------------------|-------|
| $\begin{array}{c} \text{H}_2\text{C} \text{---} \text{CH}_2 \\   \\ \text{H}_2\text{C} \text{---} \text{C} \text{---} \text{CH}_2 \text{---} (\text{O} \text{---} \text{C}_2\text{H}_4)_5 \text{---} \text{oleate} \end{array}$ | 30    |
| ( $\beta$ -hydroxy- $\beta$ -ethoxy- $\beta$ -ethoxy- $\beta$ -ethoxy ethyl tetrahydrofurfuryl ether oleate)                                                                                                                    |       |

is extended through orifices into an evaporative atmosphere. The filaments thus produced are wound, or twisted and wound. Yarns, thus produced, are pliable and suitable for knitting.

*Example 11*

|                                                                                                                                                                                                                           | Parts |
|---------------------------------------------------------------------------------------------------------------------------------------------------------------------------------------------------------------------------|-------|
| $\begin{array}{c} \text{H}_2\text{C} \text{---} \text{CH}_2 \\   \\ \text{H}_2\text{C} \text{---} \text{CH}_2 \text{---} \text{O} \text{---} \text{C}_2\text{H}_4 \text{---} \text{O} \text{---} \text{CH}_2 \end{array}$ | 80    |
| ( $\beta$ -Hydroxy ethyl tetrahydrofurfuryl ether formate)                                                                                                                                                                |       |
| Water soluble cellulose ester                                                                                                                                                                                             | 45    |
|                                                                                                                                                                                                                           | 10    |

*Example 3*

|                                                                                                                                                                                                                                                                                                                                                         | Parts |
|---------------------------------------------------------------------------------------------------------------------------------------------------------------------------------------------------------------------------------------------------------------------------------------------------------------------------------------------------------|-------|
| $\begin{array}{c} \text{H}_2\text{C} \text{---} \text{CH}_2 \text{---} \text{O} \text{---} \text{CH}_2 \text{---} \text{C} \text{---} \text{CH}_2 \text{---} (\text{O} \text{---} \text{C}_2\text{H}_4)_2 \text{---} \text{O} \text{---} \text{C} \text{---} \text{CH}_2 \text{---} \text{O} \text{---} \text{CH}_2 \text{---} \text{CH}_2 \end{array}$ | 50    |
| ( $\beta$ -hydroxy- $\beta$ -ethoxy- $\beta$ -ethoxy- $\beta$ -ethoxy- $\beta$ -ethoxy tetrahydrofurfuryl ethyl ether bis methoxy acetate)                                                                                                                                                                                                              |       |
| Blown olive oil                                                                                                                                                                                                                                                                                                                                         | 60    |

*Example 4*

|                                                                                                                                                                                                                                                                                                                                                                                                                                              | Parts |
|----------------------------------------------------------------------------------------------------------------------------------------------------------------------------------------------------------------------------------------------------------------------------------------------------------------------------------------------------------------------------------------------------------------------------------------------|-------|
| $\begin{array}{c} \text{CH}_2 \text{---} \text{CH}_2 \\   \\ \text{H}_2\text{C} \text{---} \text{CH}_2 \text{---} \text{O} \text{---} (\text{C}_2\text{H}_4)_2 \text{---} \text{O} \text{---} \text{C} \text{---} \text{C}_8\text{H}_{15} \text{---} \text{C} \text{---} \text{O} \text{---} (\text{C}_2\text{H}_4\text{---} \text{O})_2 \text{---} \text{O} \text{---} \text{CH}_2 \text{---} \text{CH} \text{---} \text{CH}_2 \end{array}$ | 55    |
| (bis( $\beta$ -hydroxy- $\beta$ -ethoxy- $\beta$ -ethoxy- $\beta$ -ethoxy tetrahydrofurfuryl ethyl ether) sebacate)                                                                                                                                                                                                                                                                                                                          |       |
| Light mineral oil                                                                                                                                                                                                                                                                                                                                                                                                                            | 60    |

*Example 5*

|                                                                                                                                                                                                                                                                                 | Parts |
|---------------------------------------------------------------------------------------------------------------------------------------------------------------------------------------------------------------------------------------------------------------------------------|-------|
| $\begin{array}{c} \text{H}_2\text{C} \text{---} \text{CH}_2 \\   \\ \text{H}_2\text{C} \text{---} \text{CH} \text{---} \text{CH}_2 \text{---} (\text{O} \text{---} \text{C}_2\text{H}_4)_5 \text{---} \text{O} \text{---} \text{C} \text{---} \text{C}_4\text{H}_9 \end{array}$ | 65    |
| ( $\beta$ -hydroxy- $\beta$ -ethoxy- $\beta$ -ethoxy- $\beta$ -ethoxy- $\beta$ -ethoxy tetrahydrofurfuryl ethyl ether valerate)                                                                                                                                                 |       |
| Blown sperm oil                                                                                                                                                                                                                                                                 | 30    |

*Example 6*

|                                                                                                                                                                                                                                                                                                                                   | Parts |
|-----------------------------------------------------------------------------------------------------------------------------------------------------------------------------------------------------------------------------------------------------------------------------------------------------------------------------------|-------|
| $\begin{array}{c} \text{H}_2\text{C} \text{---} \text{CH}_2 \\   \\ \text{H}_2\text{C} \text{---} \text{CH} \text{---} \text{CH}_2 \text{---} \text{O} \text{---} \text{C}_2\text{H}_4 \text{---} \text{O} \text{---} \text{C} \text{---} \text{C} \text{---} \text{O} \text{---} \text{CH}_2 \text{---} \text{CH}_2 \end{array}$ | 70    |
| ( $\beta$ -hydroxy ethyl tetrahydrofurfuryl ether furoate)                                                                                                                                                                                                                                                                        |       |
| Neat's-foot oil                                                                                                                                                                                                                                                                                                                   | 75    |

Any of the above compositions may be applied to the yarn intended for use in circular knitting by means of a bath, wick, spray, roller, pad or any suitable means. The amount of conditioning liquid applied may vary between 5-25% by weight of the yarn. Usually, however, the amount of conditioning liquid applied is about 10-15% by weight of the yarn. Yarn composed of cellulose acetate conditioned as described above gives excellent results when used in the circular knitting process.

As will be apparent from the above examples and description the conditioning agents of our invention may be applied by a wide variety of methods. For example, we may employ the agent

as an ingredient of the spinning dope from which the filaments are formed, the amount of the agent so employed depending upon a number of factors, such as the particular cellulose derivative used in making the yarn, the solvent or solvent combination used in making up the spinning solution, and the degree of softness or pliability desired in the yarn, etc.

If the conditioning agent is to be applied to the yarn after spinning, this may be done by bringing the yarn in contact with a wick, roll, or felt wet therewith, or the liquid may be applied by immersion, spray, or otherwise. The particular point at which the liquid is applied may vary.

15 It may, for example, be applied to the yarn inside or outside the spinning cabinet, between the guide and godet roll, between the godet or other roll or guide and the point of winding and/or twisting. In some cases, the liquid may even be applied to the yarn after winding onto cones, spools, bobbins, or the like or by the so-called "bobbin to bobbin" method. In the case of staple fiber manufacture, the liquid may be applied to the yarn prior to, or after cutting into staple lengths.

20 26 The amount of the agent so employed will vary widely depending upon the results desired, the specific nature of the material to which the agent is applied, the use to which the yarn is eventually to be put and other factors. For example, in a given case where a cellulose organic acid ester 30 yarn such as a yarn composed of cellulose acetate, is intended for knitting, about 4 to 25% or more by weight, based on the weight of the dry yarn, may be satisfactory, while if the yarn is intended 35 for weaving, the amount may vary between about 1 and 5%.

Although in the above examples we have referred primarily to yarn treating compositions containing only the conditioning agent and an oil, other ingredients such as solvents, non-solvents, emulsifying agents, blending agents and the like, may be added within the scope of our invention. Likewise, various dyes or other coloring matter may be included in case it is desired to permanently or fugitively tint or dye the material undergoing treatment.

Although we have found it convenient to illustrate our invention by reference to compositions containing specific percentages of the various ingredients, these percentages may vary widely depending upon the particular purpose for which the composition is intended. For example, if it is desired to control the solvent or softening action of the conditioning agent, the amount of the agent may be adjusted as, for example, by reducing the amount of the agent and correspondingly increasing the amount of oil or other ingredient.

While we have described our invention with particular reference to the treatment of yarns composed of organic derivatives of cellulose such as cellulose acetate, the conditioning agents and formulas described herein are applicable to the conditioning of many other types of cellulose derivative yarns such as those composed of or containing cellulose propionate, cellulose butyrate, cellulose acetate propionate, cellulose acetate butyrate, ethyl cellulose, methyl cellulose, benzyl cellulose and others, as well as to the conditioning of silk, wool, cotton, viscose and other natural or artificial materials.

The term "yarn" as used herein and in the claims is to be understood as including a single filament, a plurality of filaments associated into the form of a thread, either of high or low twist,

single or multiple threads associated or twisted together, composite threads composed of a mixture of natural and artificial filaments or a composite thread formed by twisting together individual strands of natural or artificial materials, as well as cut staple fibers produced from natural and/or artificial filaments or threads and spun yarn produced from such staple fibers.

As indicated above, the yarn conditioning agents of our invention are exceptionally good solvents for a wide variety of mineral, blown and unblown, drying and semi-drying animal and vegetable oils such as cottonseed, olive, castor, neat's-foot, sperm and other oils. This enables them to be used with any of such oils in making up a variety of yarn treating formulas of varying composition.

The yarn conditioning method and compositions of our invention possess many outstanding advantages. The fundamental and outstanding characteristic of the agents employed in accordance with the invention is their ability to soften yarns, especially those composed of or containing organic derivatives of cellulose such as cellulose acetate and render them soft and pliable and amenable to various textile operations, especially operations such as those involved in weaving and knitting where complicated designs or stitches are employed, without too drastic an action on the yarn material. Another outstanding characteristic of these compounds is their exceptional solvent power for a wide variety of mineral, animal, and vegetable oils and their ability to act as lubricating assistants in conjunction with these oils when applied to such yarns. In addition, due to their solubility in water, they may be readily removed from yarns and fabrics by means of the usual aqueous scour baths. By employing the yarn conditioning agents and method of our invention as herein described, one is enabled to obtain highly satisfactory results in the manufacture of yarns and woven fabrics and especially the production from these yarns of closely knit fabrics free from defects such as pin holes, stitch distortion, laddering and the like.

## USE OF COMPOUNDS AS PLASTICIZERS

The following examples illustrate preferred compounds in which the above mentioned compounds are employed in accordance with our invention:

### Example 12

Example 12

|                                                                                                           |                          |
|-----------------------------------------------------------------------------------------------------------|--------------------------|
| Cellulose acetate<br> | Parts<br>100<br>60<br>55 |
| ( Diethylene glycol tetrahydrofurfuryl ether phthalate )                                                  |                          |

---

### Example 13

*Example 13*

66

Cellulose acetate

$\text{H}_2\text{C}-\text{C}-\text{CH}_2$

$\text{CH}_3-\text{C}-\text{C}-\text{CH}_2-\text{O}-\text{C}_2\text{H}_4-\text{O}-\text{C}_2\text{H}_4-\text{O}-\text{C}(=\text{O})-\text{CH}_2-\text{CH}_2-$

(Diethylene glycol tetrahydrofurfuryl ether adipate)

100

40

65

**Example 14**

| Example 14                                              |     |
|---------------------------------------------------------|-----|
| Cellulose acetate                                       | 100 |
|                                                         | 70  |
| (Triethylene glycol tetrahydrofurfuryl ether succinate) | 30  |
| Ethylene chloride                                       | 300 |
| Dioxane                                                 | 100 |

**Example 15**

|                                                                      |             |
|----------------------------------------------------------------------|-------------|
| Cellulose acetate                                                    | Part<br>100 |
| 5                                                                    | 20          |
| ( $\beta$ -Hydroxy ethyl tetrahydrofurfuryl ether tetrahydrofuroate) |             |
| Triphenyl phosphate                                                  | 20          |
| 10 Acetone                                                           | 300         |
| Ethyl acetate                                                        | 100         |

*Example 16*

|                                                                                   |     |
|-----------------------------------------------------------------------------------|-----|
| Cellulose acetate propionate                                                      | 100 |
| <b>15</b>                                                                         |     |
|  | 20  |
| (Tetraethylene glycol tetrahydrofurfuryl ether acetate)                           |     |
| Butyl phthalate                                                                   | 20  |
| Ethyl lactate                                                                     | 100 |
| <b>20</b>                                                                         |     |
| Acetone                                                                           | 100 |

*Example 17*

|    |                                                                |     |
|----|----------------------------------------------------------------|-----|
| 25 | Cellulose nitrate                                              | 100 |
|    |                                                                |     |
| 30 | (Triethylene glycol tetrahydrofurfuryl ether benzyloxyacetate) | 30  |
|    | Ester gum                                                      | 40  |
|    | Ethyl acetate                                                  | 200 |
|    | Toluene                                                        | 100 |
|    | Ethanol                                                        | 100 |

### Example 18

|                    |                                                               |     |
|--------------------|---------------------------------------------------------------|-----|
| Cellulose butyrate | 100                                                           |     |
| 35                 |                                                               | 40  |
|                    | (Ethylene glycol tetrahydrofurfuryl ether tetrahydrobenzoate) |     |
| 40                 | Ethylene chloride                                             | 300 |
|                    | Acetone                                                       | 100 |

*Example 19*

|    |                                                                                     |     |
|----|-------------------------------------------------------------------------------------|-----|
| 45 | Cellulose acetate butyrate                                                          | 100 |
|    |  | 20  |
|    | (Penta ethylene glycol tetrahydrofurfuryl ether laurate)                            |     |
|    | Triphenyl thiophosphate                                                             | 20  |
| 50 | Ethylene chloride                                                                   | 400 |
|    | Methanol                                                                            | 100 |
|    |                                                                                     | 100 |

### Example 20

|                                                                                                                                                                                                                             |       |
|-----------------------------------------------------------------------------------------------------------------------------------------------------------------------------------------------------------------------------|-------|
| Ethyl cellulose.....                                                                                                                                                                                                        | 100   |
| 55 $\text{CH}_3-\text{O}-\text{CH}_2-\text{C}(=\text{O})-\text{O}-\text{CH}_2-\text{CH}(\text{O}-\text{CH}_2-\text{CH}_2-\text{O}-\text{C}_2\text{H}_5-\text{O}-\text{C}(=\text{O})-\text{CH}_2-\text{O}-\text{CH}_3$ ..... | 40 55 |
| Acetone.....                                                                                                                                                                                                                | 400   |

included within the scope of the claims appended hereto.

### What we claim is:

1. The process of conditioning yarn to render it more amenable to textile operations including knitting, weaving, spinning and the like which comprises applying thereto a lubricating and softening composition containing as its essential lubricating and softening component an ester of a hydroxyalkoxy tetrahydrofurfuryl ether having the formula:



where  $n$  is a small whole number at least one.

## 2. The process of conditioning yarn composed 75

of or containing organic derivatives of cellulose to render it more amenable to textile operations including knitting, weaving, spinning and the like which comprises applying thereto a lubricating and softening composition containing as its essential lubricating and softening component an ester of a hydroxyalkoxy tetrahydrofurfuryl ether having the formula:



where  $n$  is a small whole number at least one.

3. The process of conditioning yarn composed  
5 of or containing cellulose acetate to render it  
more amenable to textile operations including  
knitting, weaving, spinning and the like, which  
comprises applying thereto a lubricating and  
softening composition containing as its essential  
0 lubricating and softening component an ester of  
a hydroxyalkoxy tetrahydrofurfuryl ether having  
the formula:



where  $n$  is a small whole number at least one.

4. The process of conditioning yarn composed of or containing cellulose acetate to render it more amenable to textile operations including knitting, weaving, spinning, and the like, which comprises applying thereto a lubricating and softening composition containing as its essential lubricating and softening component an ester of a hydroxylalkoxy tetrahydrofurfuryl ether having the formula:



where  $n$  is a small whole number at least one, and a textile lubricant.

5. Textile yarns amenable to textile operations including knitting, weaving, spinning, and the like, impregnated with a lubricant containing as its essential lubricating and softening component an ester of a hydroxyalkoxy tetrahydrofurfuryl ether having the formula:



where  $n$  is a small whole number at least one.

6. Textile yarns composed of or containing organic derivatives of cellulose amenable to textile operations including knitting, weaving, spinning and the like, impregnated with a conditioning agent comprising an ester of a hydroxylalkoxy tetrahydrofurfuryl ether having the formula:



20

where  $n$  is a small whole number at least one.

7. Textile yarns composed of or containing organic derivatives of cellulose amenable to textile operations including knitting, weaving, spinning and the like, impregnated with a conditioning agent comprising an ester of a hydroxyalkoxy tetrahydrofurfuryl ether having the formula:



35

where  $n$  is a small whole number at least one, and a textile lubricant.

JOSEPH B. DICKEY.  
JAMES G. McNALLY.